

## UNITED STATES PATENT OFFICE

2,661,387

POROUS ELECTRODE PLATES AND PROCESS  
FOR MAKING SUCH ARTICLESKarl Ackermann, Mannheim, and Leo Schlecht,  
Ludwigshafen (Rhine), Germany, assignors to  
Badische Anilin- & Soda-Fabrik Aktiengesell-  
schaft, Ludwigshafen am Rhine, GermanyNo Drawing. Application August 19, 1950,  
Serial No. 180,498Claims priority, application Germany  
September 10, 1949

6 Claims. (Cl. 136—25)

1

The present invention relates to improvements in the production of porous shaped articles.

In the production of porous shaped articles by sintering finely divided metals it is often desirable to obtain sintered bodies having the highest possible porosity. The pore volume of the sintered body is dependent in particular on the piled-weight of the powder used for sintering.

It has already been proposed, for the purpose of reducing the piled-weight and increasing the pore volume, to incorporate with the metal powder to be sintered, light metal oxide powders which are reduced to metal if the sintering is carried out in a reducing atmosphere, or to add substances which are volatilised when heated and thus act as swelling means. These methods are not capable of general employment, however, because in many cases the substances used for loosening leave behind undesirable residues or have an otherwise injurious effect.

We have now found that a loosening of the powder mass, in so far as it is magnetisable, can be obtained in a simple manner by subjecting the powder before or during the sintering to the action of a magnetic field. By this magnetic treatment, a metal powder having too high a piled-weight can be loosened to such an extent that it yields sufficiently porous shaped articles. Thus by the method according to the invention it is no longer necessary to use specially light kinds of powder or to add the above-mentioned additional substances.

When a flat mould is filled with the magnetisable powder and the powder is covered with a cover consisting of non-magnetisable material and laid loosely thereon, and the mould is then brought in a horizontal position into a strong, vertically-acting magnetic field, the cover lifts by reason of the increase in volume of the powder mass brought about by the magnetic orientation of the powder particles. At the end of the magnetic action, the increase in volume of the powder mass reverts somewhat, but there still remains a considerable loosening so that, upon sintering, shaped articles having a substantially increased pore volume are obtained. The sintering of the powder may also be carried out under the action of the magnetic field; the magnetic field need only be maintained until the powder particles have been fixed in their position by being fritted together.

Our process is applicable not only to powders consisting entirely of magnetisable particles, such as the metals and metal oxides of the iron group, but in many cases mixtures of magnet-

2

isable and non-magnetisable powders may be successfully worked up into porous shaped articles.

The invention is especially suitable for the preparation of porous electrode plates consisting of metals of the iron group, for alkaline accumulators in which the highest possible pore volume is desirable. Moreover, the pores of plates produced according to our process show an orientation in the direction towards the plate surface, and also this structure makes the plates especially convenient to the employment for the said electrode purposes.

The following example will further illustrate the invention but the invention is not restricted to this example.

## Example

A flat mould consisting of sheet chromium-nickel and having a base about 200 x 100 millimetres and a height of 18 millimetres is filled up to a height of 10 millimetres with a fine nickel powder prepared by decomposition of nickel carbonyl and the layer of powder is covered with a sheet chromium-nickel cover. The mould is brought in a horizontal position into the vertically directed field of an electromagnet so that the lines of magnetic force pass through the mould perpendicular thereto. Under the action of the magnetic field the powder mass extends in the direction of the lines of magnetic force and the applied cover is accordingly displaced upwards. The loosening of the powder remains to a great extent after the magnetic field has been switched off. The mould is then heated for 1½ hours at a temperature of 950° C. The pore volume of the sinter body thus formed amounts to about 84%, while a sinter body prepared without the aforesaid magnetic pretreatment of the powder but in otherwise an identical way has a pore volume of only 80%. The volume occupied by the nickel metal in the sinter body is thus reduced from 20% to 16% by the magnetic pretreatment. This represents a saving of nickel of 20%.

The thus obtained nickel plate is well suited as a porous electrode for alkaline accumulators.

## What we claim is:

1. An improvement in producing porous, shaped articles by sintering magnetizable materials which comprises subjecting a mass of magnetizable particles to the flux lines of a magnetic field thereby causing alignment of said particles along the flux lines and then sintering the thus

ned particles thereby forming a sintered article of increased porosity.

A process in accordance with claim 1 where-  
the particle mixture includes particles of a  
magnetizable metal and particles of a non-mag-  
netizable substance.

A process in accordance with claim 1 where-  
the particle mixture includes particles of a  
magnetizable metal oxide and particles of a non-  
magnetizable substance.

An improvement in the production of porous  
articles by sintering powders of magnetizable ma-  
terials which comprises arranging a mass of the  
powder in a flat mold, positioning the mold hori-  
zontally in a vertically directed field of an elec-  
tromagnet so that the lines of magnetic force  
pass through the mold perpendicularly thereto,  
switching off the magnetic field and then sinter-  
ing the mass to which an increased porosity has  
been imparted by the aforesaid magnetic treat-  
ment.

An improvement in producing porous plates  
by sintering magnetizable powdered materials  
which comprises forming a flat mass of the  
powder into a plate form, positioning said plate  
horizontally in the vertically directed field  
of an electro-magnet so that the lines of mag-  
netic force pass through said form perpendi-

cularly thereto thereby causing the particles to  
align in the path of the lines of the magnetic  
force, switching off the magnetic field and then  
sintering the mass.

5 As a new article of manufacture, porous  
electro-plates for alkaline accumulators, the  
pores of said plates being oriented in the direc-  
tion towards the plate surface, said orientation  
being effectuated by shaping a mass of magnet-  
izable particles into the form of a plate, position-  
ing the aforesaid plate-shaped mass in a  
magnetic field wherein the lines of magnetic flux  
pass transversely of said plate thereby to align  
the particles thereof and after said alignment  
10 sintering the same.

KARL ACKERMANN.  
LEO SCHLECHT.

## References Cited in the file of this patent

## UNITED STATES PATENTS

| Number       | Name             | Date           |
|--------------|------------------|----------------|
| 1,878,713    | Roseby           | Sept. 20, 1932 |
| 25 1,942,791 | Ackerman         | Jan. 9, 1934   |
| 1,981,468    | Roseby           | Nov. 20, 1934  |
| 1,988,861    | Thorausch et al. | Jan. 22, 1935  |
| 2,188,091    | Baermann, Jr.    | Jan. 23, 1940  |